

# United States Patent [19]

Lutz et al.

[11] 3,892,557

[45] July 1, 1975

[54] **PROCESS FOR THE PRODUCTION OF GOLD POWDER IN PLATELET FORM**

[75] Inventors: **Klaus Lutz, Bergen-Enkheim; Manfred Golla, Grossauheim, both of Germany**  
[73] Assignee: **Demetron Gesellschaft fur Elecktronik-Werkstoffe mbH, Frankfurt, Germany**

[22] Filed: **May 31, 1974**

[21] Appl. No.: **475,280**

[30] **Foreign Application Priority Data**

June 15, 1973 Germany..... 2330413

[52] U.S. Cl. .... **75/0.5 A; 75/118 R**

[51] Int. Cl. .... **C22b 11/06**

[58] **Field of Search..... 75/0.5 A, 118**

[56]

**References Cited**

**UNITED STATES PATENTS**

|           |        |                    |          |
|-----------|--------|--------------------|----------|
| 3,201,223 | 8/1965 | Cuhra et al .....  | 75/118   |
| 3,401,186 | 9/1968 | Muller et al ..... | 75/118   |
| 3,717,453 | 2/1973 | Daiga.....         | 75/0.5 A |
| 3,725,035 | 4/1973 | Short et al .....  | 75/118   |
| 3,725,047 | 4/1973 | Schneider .....    | 75/118   |

*Primary Examiner*—W. Stallard

*Attorney, Agent, or Firm*—Cushman, Darby & Cushman

[57] **ABSTRACT**

Gold powder is produced in flake form by reducing aqueous hydrochloric acid solution of chloroauric III acid with an unsaturated alcohol in the presence of a protective colloid.

**9 Claims, No Drawings**

## PROCESS FOR THE PRODUCTION OF GOLD POWDER IN PLATELET FORM

The invention concerns a process for the production of flake (platelet) gold powder by reduction of aqueous hydrochloric acid solutions of chloroauric (III) acid ( $\text{HAuCl}_4$ ) with unsaturated alcohols, i.e., ethylenically or acetylenically unsaturated alcohols, in the presence of a protective colloid.

Gold powder of various particle sizes and shapes is employed in many areas of the arts, as for example, for the production of decorative articles, electrical conductors and resistances, or for printed circuits.

In the previously known process for the production of gold powders by the reduction of gold salt solutions with chemical reducing agents, the powder forms as irregular particles, frequently even as needles. In the industrial use of gold powder, especially for conductive pastes, however, it has been shown that flake particles are better suited for such purposes than powders which consist of other particle forms. For the production of flake type gold powder, customarily crystalline powder is started with and it is ground with steel balls in a ball mill for a long time. Suitably, there are added grinding assisting agents as, for example, fatty acids or organic hydrocarbon. Short U.S. Pat. No. 3,539,114. Because of the ductility of the gold, the starting crystallites are shaped thereby to more or less large flakes. However, these processes have the disadvantage that they are very time-consuming and a product is produced that does not fulfill all of the requirements placed on a true flake form of gold powder.

Therefore, it was the problem of the present invention to find a process which permits the direct production in a chemical way of a flake form of gold powder directly from the solution of a gold salt.

It has now been found according to the invention that there can be obtained well formed, flake gold powder directly by reduction of gold solutions if one starts with an aqueous, hydrochloric acid solution of chloroauric (III) acid and reduces this with an ethylenically or acetylenically unsaturated alcohol in the presence of a protective colloid.

As the protective colloid there is preferably used gum arabic in an amount of 2 to 6% of the mixture. However, there can also be used other colloid constituents such as dextrin methyl cellulose, tannic acid, gum tragacanth, sodium alginate, potassium alginate, gelatin, kolophonium etc. The amount of protective colloid can also range from 2 to 15 % of the weight of the mixture.

As the reducing agent there can be used any ethylenically or acetylenically unsaturated alcohol, e.g., alkenols such as allyl alcohol, methallyl alcohol, crotyl alcohol, oleyl alcohol, linolyl alcohol or alkinols such as propargyl alcohol or citronellol.

Especially valuable are alcohols having a double bond (or triple bond) in the alpha position, especially allyl alcohol and/or propargyl alcohol. There can also be used as reducing agents enediols and other organic compounds which have an OH group adjacent to a double bond.

Preferably the reduction to gold powder takes place at a pH of between 0 and 4. The hydrochloric acid solution containing chloroauric (III) acid must contain at least 5% of gold by weight. With solutions containing less than 5% gold, there is no separation of flake shaped powder. There is no critical upper limit on the amount

of gold, e.g., it can be present up to a saturated solution. By variation of the reduction parameters such as temperature or pH value, the size of the flakes can be influenced in the range of, for example, 1 to 50  $\text{m}\mu$  whereby the gold crystallizes in the form of triangular or hexagonal flakes.

Generally, the reduction takes place by slowly dropping the reducing agent into a solution mixture of chloroauric (III) acid and protective colloid. The amount of reducing agent added depends on the gold content of the solution. Preferably the amount of reducing agent, however, is greater than that stoichiometrically needed for reaction with the gold in order that the reduction is quantitative.

Very finely crystalline gold flakes are obtained if the chloroauric (III) acid solution is treated with the reducing agent at low temperatures (e.g., room temperature such as 18°-25°C.) diluted with water and the solution allowed to decolorize. Then the mixture is heated to 80°-90°C. whereupon the gold powder precipitates. The temperature can thus range from room temperature to the boiling point.

The flake shaped gold powder produced by the process of the invention is especially suited for decorative and thick film-conducting pastes because of its good screen printing properties and the high electrical conductivity of the baked conductor path.

Unless otherwise indicated, all parts and percentages are by weight.

The process of the invention will be further explained in the following examples.

### EXAMPLE 1

3.3 kg of an  $\text{HAuCl}_4$  solution containing about 33% Au was diluted with soda lye to pH 0.5-1 and treated with 2 kg of aqueous 30% gum arabic solution. There was added with stirring at a maximum temperature of 30°-35°C. 1 liter of allyl alcohol in the course of 90 minutes. The reduction mixture was held at room temperature until the first appearance of gold flakes, then warmed to 60°-70°C. and held there for about 15 minutes. The gold powder was washed by decantation with water and alcohol, filtered with suction and dried at 70°C. There was obtained thereby a quantitative yield of crystalline flakes of particle size of 25  $\text{m}\mu$  or less.

### EXAMPLE 2

A mixture of 750 ml of allyl alcohol and 250 ml of propargyl alcohol was dropped into a mixture of 3.3 kg of 30% aqueous  $\text{HAuCl}_4$  solution (pH 1-1.5) and 2 kg of aqueous 30% gum arabic solution with stirring at 70°-80°C. within 90 minutes. Further reaction was allowed to continue for 10 minutes at this temperature. There were obtained thereby crystalline flakes having a particle size of not over 15  $\text{m}\mu$ .

### EXAMPLE 3

To 1.6 kg of an aqueous  $\text{HAuCl}_4$  solution (pH 1-1.5) and 1 kg of a 30% aqueous gum arabic solution there were dropped in a mixture of 500 ml of allyl alcohol and 500 ml of water at 50°-60°C. during 4 hours. There were obtained crystalline flakes of particle size of 2 to 50  $\text{m}\mu$ .

### EXAMPLE 4

A mixture of 3.3 kg of aqueous  $\text{HAuCl}_4$  solution (pH 1), 2 kg of 30% aqueous gum arabic solution and 1 liter

of allyl alcohol were diluted with water in the ratio of 1:1 by volume. The mixture was held with stirring at a maximum temperature of 30°C. until the solution had decolorized. Then it was warmed to 80°C. and there was obtained a gold powder which consisted of flakes having a particle size of 5  $\mu\text{m}$  or less.

EXAMPLE 5

3.3 kg of an aqueous  $\text{HAuCl}_4$  solution containing about 33 % Au was diluted with a 10 % aqueous solution of NaOH to pH 5 and treated with 1.2 kg of an aqueous 30 % dextrose solution. There was dropwise added 1 kg ascorbic acid to this mixture. There was obtained thereby crystalline flakes of particle size of 10 – 60  $\mu\text{m}$ .

EXAMPLE 6

3.3 kg of an aqueous  $\text{HAuCl}_4$  solution (pH 1) was treated with 1.5 kg of 30 % aqueous dextrose solution. This mixture was reduced with 2 kg butane-2-ol by boiling. There was obtained thereby crystalline flakes of particle size of 5 – 10  $\mu\text{m}$ .

What is claimed is:

1. A process for the production of gold powder in

25

flake form comprising reducing an aqueous hydrochloric acid solution of chloroauric (III) acid with an ethylenically or acetylenically unsaturated alcohol in the presence of a protective colloid.

2. A process according to claim 1 wherein the alcohol is an alkenol.

3. A process according to claim 1 wherein the alcohol is an alkyneol.

4. A process according to claim 1 wherein the alcohol is an alkeneol or alkyneol and the hydroxyl group is attached to a carbon atom alpha to a carbon atom containing the ethylenic or acetylenic unsaturation.

5. A process according to claim 1 wherein the solution has a pH between 0 and 4.

15 6. A process according to claim 5 wherein the protective colloid is gum arabic.

7. A process according to claim 6 wherein the reducing agent is allyl alcohol, propargyl alcohol or a mixture of allyl alcohol and propargyl alcohol.

8. A process according to claim 5 wherein the unsaturated alcohol is allyl alcohol.

9. A process according to claim 5 wherein the unsaturated alcohol is propargyl alcohol.

\* \* \* \* \*

30

35

40

45

50

55

60

65